

July 8, 1924.

1,500,097

C. D. ABRAHAM

IMPERVIOUS SEAMED ARTICLE AND PROCESS OF MAKING THE SAME

Filed April 14, 1920



Fig. 1



Fig. 2

C. D. Abraham, Inventor

By his attorney J. R. Squair.

Patented July 8, 1924.

1,500,097

# UNITED STATES PATENT OFFICE.

CLINTON D. ABRAHAM, OF WILMINGTON, DELAWARE; CHESTER H. ROSS ADMINISTRATOR OF SAID ABRAHAM, DECEASED.

## IMPERVIOUS-SEAMED ARTICLE AND PROCESS OF MAKING THE SAME

Application filed April 14, 1920. Serial No. 373,961.

To all whom it may concern:

Be it known that I, CLINTON D. ABRAHAM, a citizen of the United States, and a resident of Wilmington, in the county of New Castle and State of Delaware, have invented certain new and useful Impervious-Seamed Articles and Processes of Making the Same, of which the following is a specification.

10 This invention relates to seamed articles, more particularly to articles of wearing apparel, which are impervious and resistant to acids, poisonous gases, and various other chemical reagents, against which ordinary apparel affords but slight protection; the invention also relates to a process of making such articles, and also to a coating composition useful in the making of such articles. By the term "seamed" I do not refer merely 15 to articles having their parts joined by sewing, but mean also articles whose parts are joined in any other suitable and similar manner as, say, by spaced fasteners or the like. The invention finds advantageous application in the field of acid resistant gloves, and, so, for the sake of definiteness I describe it with more particular reference to 20 such gloves, but do not restrict it thereto.

Protective gloves have heretofore been 25 made of rubber; the practice of the rubber trade in this connection has been to dip porcelain forms repeatedly into rubber cement until the proper thickness of film has been built up, and then to cure the rubber 30 in sulfur chloride solution, thereby producing an all-rubber product. According to another method the gloves are built up of 35 rubberized stockinet in the manner of overshoes, by cementing pieces together.

40 The above-mentioned old methods have certain disadvantages which it is one of the objects of my invention to avoid. The porcelain form which is used in making the all-rubber product is difficult to remove from 45 the rubber coating which has been built thereon. The all-rubber glove is expensive, and is not suitable as a protective covering against certain kinds of poisonous gases.

The gloves built up of rubberized stockinet 50 are not sufficiently strong and durable. The seams constitute the weak portions of such gloves, it being difficult to render these portions as strong and resistant to penetration by liquids as the rest of the glove.

55 Also, it has been proposed, in the making

of certain seamed articles, to immerse the goods from which the article is to be made, in a bath to impregnate and saturate the goods, to then sew certain parts of the article together, and to then apply by hand a 60 coat of varnish which extends into and across the lines along which the said certain parts of the article are sewed together; but this proposed procedure involved, among other difficulties, the difficulty that the immersion in the bath treated 65 the back of the goods, and also the difficulty that the applying of the varnish by hand was a time-consuming labor not to be thought of when one wished to produce a 70 large number of articles by "quantity production" methods. Varnishing the back of the goods—the side that, in articles of wearing apparel, as gloves, is the inside—would render the back not well suited for contact 75 with the flesh of the wearer.

I have devised a seamed article, more particularly a glove, in which the various difficulties of prior articles are avoided; have devised a process for the making of such 80 articles, and have also devised a coating composition useful in the carrying out of my process, to produce the articles.

One of the objects of my invention is to provide a seamed article in which various 85 of the disadvantages of previous articles are obviated; and, more particularly, is to provide a glove which shall be comfortable to the hand, have its seams well closed, can be readily manufactured in quantity, and shall 90 be impervious and resistant to acids, gases and so forth.

Another object is to provide a process by which articles, more particularly gloves, embodying my invention, can be produced expeditiously and comparatively inexpensively.

Another object is to provide a coating composition useful in the carrying out of my process to produce my article.

To these and other ends, and also to improve generally upon articles, processes, and compositions, of the character indicated, my invention consists in the following matters hereinafter described and claimed.

In the accompanying drawing, Figure 1 105 is a plan view of a glove embodying the invention as it relates to articles, and produced in accordance with the present process, with the various coatings broken back to show the fabric, and Figure 2 is an enlarged con- 110

ventional cross-sectional view taken at one of the seams of the glove.

Speaking generally, my process, as preferably practiced in the making of gloves, 5 comprises applying to one side only of a web of fabric 1, preferably composed of cotton, one or more coatings of a solution of a film-forming material resistant and impervious to acids and gases. The coated fabric, after 10 drying to provide the film 2, is then cut up and the parts sewed together as indicated at S to make up the gloves, complete. The gloves are then placed, with the coated side exposed, on suitable forms, of a shape to 15 cause the gloves to present a smooth surface, and dipped into a solution similar to that employed in coating the fabric. After removing the gloves from the solution, and drying them, the dipping and the drying of 20 them are preferably repeated one or more times to thoroughly cover all seams and cracks with the film 3.

It will be noted that, by proceeding in the manner above outlined, I am enabled to arrive at certain valuable results:—Since I 25 coat the fabric, as distinguished from submerging it in a bath, and coat it, too, upon but one side, I preserve the other side of the fabric in a proper condition to be worn next 30 the hand, e. g. preserve the nap. By making up the glove completely, that is putting all the fabric parts together and forming the seams, before the dipping operations, I get, after the dipping, a glove with all the seams 35 protected. By coating the fabric while it is in the web I am able to put on much of the necessary protection when the fabric is in a form to be conveniently and expeditiously handled by machine methods. And by applying the final coats by dipping, as distinguished 40 from applying by hand, I am able to treat a large number of the gloves at a time by machine methods. Thus the process lends itself to the expeditious and inexpensive production of the article in large 45 quantities. Of course, too, the use of the fabric base eliminates all troubles, such as difficulty in removing the gloves from the forms, and the like.

50 One of the preferred ways of carrying out my new process as applied to gloves is illustrated by the following example:—

The fabric from which the gloves are to be made should have a smooth surface on one 55 side in order that it may be given a smooth, even coating. The other side should have a soft, napped finish for warmth and comfort against the hand. The cloth best suited for this purpose is a twill weave, cotton fabric, commonly known as sateen. It has a count of 93 x 64 and weighs 8.2 oz. per square yard.

After one side of this fabric has been given a soft, napped finish by running over revolving wire brushes, it is coated on the

smooth side with a solution of a material resistant and impervious to acids and gases, the composition of which is hereinafter described.

Four coats are applied by running the 70 fabric through a spreading machine of conventional design, using a sharp knife blade in applying the first two coats and a blade with rounded edge for the last two. This treatment makes difficult the penetration of 75 the fabric by the solution in which it is subsequently dipped.

The material thus coated is cut into proper shape by dies and made up into 80 gloves. For this purpose I prefer a mitten having a separate thumb and index finger and provided with a cuff at least six inches long.

The gloves are then placed on wooden 85 forms so constructed as to extend the finger and thumb and present a smooth surface without wrinkles. The form is then attached to a rack and lowered into a solution of the same nature as that used to coat the fabric.

90 After immersion in the solution the gloves are inverted and passed through a heated drying chamber. When dried they are given a second coat.

The gloves are preferably given two or 95 more dip coats to thoroughly cover all seams and cracks. They are then removed from the forms and allowed to dry thoroughly at room temperature.

The coating solution which is spread on 100 the fabric before the latter is made up into gloves, may have the following composition (parts are by weight in each instance):—

#### Heavy bodied boiled

|             |    |   |               |        |                          |
|-------------|----|---|---------------|--------|--------------------------|
| Linseed oil | 65 | — | 85            | parts. | 105.                     |
| Lamp black  | 5  | — | 20            | parts. |                          |
| Castor oil  | 2  | — | 15            | parts. |                          |
| Paraffin    | 2  | — | 15            | parts. |                          |
| Litharge    | —  | — | $\frac{1}{4}$ | —      | $\frac{3}{4}$ of a part. |
| Raw umber   | —  | — | $\frac{1}{4}$ | —      | $\frac{3}{4}$ of a part. |
| Gasoline    | 60 | — | 150           | parts. | 110                      |

I have found a solution of the following composition to be suitable in this connection:—

|             |   |               |            |
|-------------|---|---------------|------------|
| Linseed oil | — | 79            | parts.     |
| Lamp black  | — | 10            | parts.     |
| Castor oil  | — | 5             | parts.     |
| Paraffin    | — | 5             | parts.     |
| Litharge    | — | $\frac{1}{2}$ | of a part. |
| Raw umber   | — | $\frac{1}{2}$ | of a part. |
| Gasoline    | — | 80            | parts.     |

The solution in which the gloves are 125 dipped desirably has the same ingredients in substantially the same proportions as in the just above formula except that more solvent is used, desirably 100 parts of gasoline.

The above composition contains, it will be 130

noted, castor oil as a softener. Such a composition including a drying oil and a softening oil, has certain advantages, and I include such a composition within my invention as 5 a feature thereof.

It will be understood that other materials than those given above can be used, say drying oils similar to linseed, as China wood oil, or rubber, and I consider these and 10 characteristically similar materials as within my invention.

For rubber, for the initial coating solution spread in the goods before they are made up, I suggest:—

|    |                 |    |   |     |        |
|----|-----------------|----|---|-----|--------|
| 15 | Crude rubber    | 25 | — | 75  | parts. |
|    | Lamp black      | 3  | — | 15  | parts. |
|    | Litharge        | 10 | — | 50  | parts. |
|    | Natural bitumen | 2  | — | 10  | parts. |
| 20 | Paraffin        | 1  | — | 5   | parts. |
|    | Barytes         | 3  | — | 15  | parts. |
|    | Sulphur         | 2  | — | 2½  | parts  |
|    | Gasoline        | 83 | — | 200 | parts. |

Specifically, I have found a solution of 25 the following composition to be suitable:—

|    |                 |     |        |
|----|-----------------|-----|--------|
|    | Crude rubber    | 50  | parts. |
|    | Lamp black      | 10  | parts. |
|    | Litharge        | 25  | parts. |
| 30 | Natural bitumen | 5   | parts. |
|    | Paraffin        | 1½  | parts. |
|    | Barytes         | 7   | parts. |
|    | Sulphur         | 1½  | parts. |
|    | Gasoline        | 125 | parts. |

35 Comparable to the case of linseed oil, the solution in which the gloves are dipped desirably has the same ingredients in substantially the same proportions as in the just above formula except that more solvent is 40 used, desirably 150 parts of gasoline.

Men wearing gloves made by this method can safely handle poisonous and corrosive solids, liquids and gases. Gloves can be made by this method much more rapidly and 45 economically than by the methods commonly used in making acid proof gloves.

As will be evident from the above description, the new protective gloves may be said to comprise several pieces of suitably shaped 50 fabric 1 preliminarily coated on one side with a composition 2 that resists acids and gases, said pieces being sewed together as at S, and being covered on that same said side with an additional layer 3 of a composition 55 of similar characteristics, applied after the several pieces of fabric have been joined. The exterior surface of the glove is therefore a continuous film unbroken at the seams.

60 The margin of the several pieces of fabric, that is the portion lying between the edge of the pieces of fabric and the seams, will not be exposed to the solutions in which the assembled glove is dipped, and consequently 65 the layer of composition on said margins

will not be as thick as the layer of composition which constitutes the outside surface of the glove.

Although I have above described the coating of the glove with two substantially like 70 films, as two oil films, or two rubber films, it will be understood that if desired, I may use films that are not the same, though they are essentially similar in both being impervious and resistant. That is, I may use first 75 an oil film on the fabric before the making up of the glove, and then may use a rubber film after the glove is made up, or vice-versa.

While the invention has been described 80 in considerable detail it will be understood that the specific examples given are merely illustrative and that various changes may be made therein without departing from the spirit and scope of my invention. 85

As will be understood, a rubber film is cured after drying, either in a hot air oven for two hours at a temperature of about 250° F. or by dipping into a solution of sulphur-chloride dissolved in carbon tetrachloride or other suitable solvents such as carbon disulphide or benzol. In cases where the sulphur-chloride cure is to be used the sulphur is omitted from the formula for the rubber. Where oven curing is used it 90 preferably occurs after both films have been applied, not only in the cases where both are rubber or only the outer of rubber, but also where the outer film is of oil; where the sulphur-chloride cure is used and the outer film is oil the curing is done before the outer film is applied. In applying the various coats making up the two films, each coat is preferably dried before applying the next. 100

105 I claim

1. The process of making an impervious seamed article which comprises securing together the margins of suitably shaped fabric that has been coated on one side only with an impervious film, applying a coating solution of an impervious film-forming substance to the resulting article, and upon said one side only, and drying the article to produce a second film. 110

2. The process of making an impervious seamed article, of wearing apparel, which comprises securing together the margins of suitably shaped fabric that has been coated on one side only with an impervious film, applying a coating solution of an impervious film-forming substance to the resulting article, and upon said one side only, and over the entire surface of such side and drying the article to produce a second film. 120

3. The process of making an impervious seamed article, which comprises securing together the margins of suitably shaped fabric which has been napped on the one side, and coated on the other side only with an 125

- impervious film, applying a coating solution of an impervious film-forming substance to the resulting article and upon the coated side only, and drying the article to produce 5 a second film.
4. The process of making an impervious seamed article, which comprises applying an impervious film to one side only of a web of fabric, making the fabric into article 10 form, such step including joining certain of the margins of the fabric, dipping the article, with said one side only exposed, in a solution of an impervious film-forming substance, and drying the article.
- 15 5. The process of making an impervious seamed article which comprises securing together the margins of suitably shaped fabric that has been coated on one side only with an impervious film, applying a coating solution 20 of an impervious film-forming substance to the resulting article, and drying the article to produce a second film; one of said films comprising linseed oil.
- 25 6. The process of making an impervious seamed article which comprises securing together the margins of suitably shaped fabric that has been coated with an impervious film, applying a coating solution of an impervious film-forming substance to the resulting 30 article, and drying the article to produce a second film; one of said films comprising rubber.
- 35 7. The process of making an impervious seamed article which comprises securing together the margins of suitably shaped fabric that has been coated with an impervious film, applying a coating solution of an impervious film-forming substance to the resulting article, and drying the article to 40 produce a second film; one of said films comprising linseed oil and a softener therefor.
- 45 8. The process of making an impervious seamed article, which comprises securing together the margins of suitably shaped fabric that has been treated on one side only with a coating solution of an impervious film-forming substance to provide a film thereon, applying to the resulting article a coating 50 solution of an impervious film-forming substance, essentially similar to the first named substance, and drying the article.
- 55 9. The process of making an impervious seamed article, which comprises securing together the margins of suitably shaped fabric that has been treated on one side only with a coating solution of an impervious film-forming substance to provide a film thereon, applying to the resulting article a coating 60 solution of an impervious film-forming substance, substantially the same as the first named substance, and drying the article.
- 65 10. The process of making an impervious article, which comprises coating a web of fabric with a solution of an impervious 70 film-forming substance, dissolved in a suitable solvent, drying the fabric to provide a film, making the fabric into the article, coating the made up article with a solution essentially similar to the first named solution though containing more solvent, and drying the article.
- 75 11. The process of making an impervious article, which comprises coating a web of fabric with a solution of an impervious film-forming substance, dissolved in a suitable solvent, drying the fabric to provide a film, making the fabric into the article, coating the made up article with a solution 80 substantially the same as the first named solution though containing more solvent, and drying the article.
- 85 12. The process of making an impervious article, which comprises coating a web of fabric with a solution of an impervious film-forming substance dissolved in a suitable solvent, drying the fabric to provide a film, making up the fabric into the article, coating the made up article with a solution 90 essentially similar to the first named solution, and drying the article; one of said solutions comprising 65 and 85 parts of linseed oil, 2 to 15 parts of castor oil and 60 to 150 parts of solvent.
- 95 13. The process of making an impervious article, which comprises coating a web of fabric with a solution of an impervious film-forming substance dissolved in a suitable solvent, drying the fabric to provide a film, making up the fabric into the article, coating the made up article with a solution 100 essentially similar to the first named solution, and drying the article; one of said solutions comprising 25 to 75 parts of crude rubber, 10 to 50 parts of an accelerator, 0 to 2½ parts of sulphur and 83 to 200 parts of solvent.
- 105 14. The process of making protective gloves which comprises applying a resistant film to one side only of a web of fabric, making up such web of fabric into gloves, immersing the so made gloves, with the coated side only exposed, in a solution of a resistant film-forming substance, and drying the gloves to produce a second film.
- 110 15. The process of making an impervious seamed article which comprises securing together the margins of suitably shaped fabric that has been coated with an impervious film, applying a coating solution of an impervious film-forming substance to the resulting article, and drying the article to produce a second film; one of said films comprising a drying oil and a softener therefor.
- 115 16. The process of making an impervious seamed article which comprises securing together the margins of suitably shaped fabric that has been coated with an impervious film, applying a coating solution of an impervious film-forming substance to the re- 120
- 125 130

sulting article, and drying the article to produce a second film; one of said films comprising a drying oil and a vegetable softener therefor.

- 5 17. The process of making an impervious seamed article which comprises securing together the margins of suitably shaped fabric that has been coated with an impervious film, applying a coating solution of an impervious film-forming substance to the resulting article, and drying the article to produce a second film; one of said films comprising a drying oil and a softener oil therefor.
- 10 18. The process of making an impervious seamed article which comprises securing together the margins of suitably shaped fabric that has been coated with an impervious film, applying a coating solution of an impervious film-forming substance to the resulting article, and drying the article to produce a second film; one of said films comprising linseed oil and castor oil.
- 15 19. A multi-part article comprising a plurality of joined pieces of textile fabric coated, on the exterior surface of the article only, with a film impervious to fluids and continuous over the surface proper and the joining lines, to be impervious to fluids over the entire exterior surface of the article, including the joining lines of said pieces.
- 20 20. A multi-part article comprising a plurality of joined pieces of textile fabric coated, on the exterior surface of the article only, with a film impervious to fluids and continuous over the surface proper and the joined margins, to be impervious to fluids over the entire exterior surface of the article, including the joined margins.
- 25 21. A multi-part article comprising a plurality of joined pieces of textile fabric coated, on the exterior surface of the article only, with a film impervious to fluids and continuous over the surface proper and the joining lines, and including a coating of rubber composition, to be impervious to fluids over the entire exterior surface of the article, including the joining lines of said pieces.
- 30 22. A seamed textile fabric article of wearing apparel composed of textile fabric joined along certain of its margins and coated, on the exterior surface of the article only, with a film impervious to fluids and continuous over the surface proper and the joined margins, to be impervious to fluids over the entire exterior surface of the article, including the joined margins.
- 35 23. A protective glove made of cotton fabric having a soft, napped interior surface and having for its exterior surface a continuous film of fluid-impervious material extending over the seams of the glove as well as over the unseamed surface thereof.

In testimony whereof I affix my signature.  
CLINTON D. ABRAHAM.